

## UNITED STATES PATENT OFFICE

GEORGE A. RICHTER, OF BERLIN, NEW HAMPSHIRE, ASSIGNOR TO BROWN COMPANY,  
OF BERLIN, NEW HAMPSHIRE, A CORPORATION OF MAINE

## PULP-TREATING PROCESS

No Drawing.

Application filed December 1, 1925. Serial No. 73,602.

This invention relates to the treatment of a sulphite pulp, which has been prepared under special conditions, to yield a product having certain optimum characteristics to be hereinafter described.

In my application, Serial No. 749,564, filed November 12, 1924, it is disclosed that when wood chips (spruce, for example) are cooked in an acid sulphite solution in which the free  $\text{SO}_2$  and the combined  $\text{SO}_2$  are present in substantially equal proportions (or the free  $\text{SO}_2$  less in proportion than combined  $\text{SO}_2$ ), but are present in sufficient proportion to the weight of the solution to act upon the encrusting or cementitious content of the wood for a sufficient period of time in a closed digester, at a temperature higher than that ordinarily employed in sulphite digestion, a pulp is produced which has unusual characteristics and which possesses features of advantage over the usual or commercial form of sulphite pulp. First, the product has longer fibers and a much greater strength than the usual commercial sulphite pulp; and, second, it is comparable in average length of fiber and strength with sulphate or kraft pulp, but has the advantages thereover, that it is not so dark in color and requires less beating to condition it for use in the manufacture of paper. A sheet formed of this pulp, with or without beating, has a shiny or glossy appearance and has a decided "rattle" when shaken. Its appearance is markedly different from that of either commercial sulphite or sulphate pulp, and as stated, it possesses the best characteristics of both sulphite and sulphate pulps in the particulars mentioned. Moreover, the new pulp contains a higher proportion of the wood than is contained in either sulphate or commercial sulphite pulp. Hence, in addition to cellulose fibers, the product contains a large proportion of lignin and pentosan, which by their presence doubtless impart to the product certain identifying characteristics hereinbefore noted.

To produce pulp such as has been described, the wood chips are cooked in an acid sulphite solution having a relatively high combined  $\text{SO}_2$  content say, 3% to 4%) with free  $\text{SO}_2$  no greater in proportion than the combined

$\text{SO}_2$ , at a temperature of about 320° F. and a total pressure of about 75 to 95 pounds. The cooking operation is carried out at this temperature and pressure for about ten to eleven hours, tests being made in the usual manner to determine the progress of the operation and to ascertain when the chips have been cooked to the desired extent. In such a process, the cellulose fibers are substantially uninjured, since the hydrolysis of the fibers is less than where there is an excess of free  $\text{SO}_2$ , and hence the average length of fiber is greater than when the acid cooking is carried on with an excess of free  $\text{SO}_2$ ; whereas, on the other hand, the pulp contains much of the fiber that in an alkaline digestion would be dissolved in the alkaline liquor.

I present herein a table which indicates the characteristics which a sulphite pulp produced by the method described possesses, these characteristics being represented by average figures obtained in testing samples from different cooks:

| Characteristics of "4-4" pulp |              |
|-------------------------------|--------------|
| Time of beating               | 50 minutes   |
| Strength (Mullen)             | 170-182      |
| Tear                          | 92-140       |
| Pentosan                      | 5.0% to 6.0% |
| Alpha cellulose               | 88%-89%      |
| Copper number                 | 2-3          |

Thus it will be seen that a surprising strength of pulp is secured, which is comparable to that of "kraft" or sulphate pulp, which usually possesses a Mullen strength (beaten) of about 155 to 165.

I have further discovered that when such sulphite pulp, herein termed a "4-4" pulp, is treated with a concentrated solution of an alkaline compound, such as caustic soda, at about room temperature, the alkaline solution containing sufficient alkali to react with the lignin, less-resistant celluloses, and certain other impurities contained in the pulp, but insufficient to cause a substantial mercerization of the alpha cellulose content thereof, the tear test of such pulp is materially increased and a product results which is especially high in alpha or resistant cellulose. In carrying out this treatment or purification of "4-4" pulp,

too high a concentration of caustic soda must be avoided, since otherwise the alpha cellulose content of the pulp will become mercerized. Mercerization tends to lower the strength of the pulp very materially, and on beating, such pulp does not tend to hydrate or jell, the beating operation merely tending to macerate or shred the fiber, and resulting in a paper of low strength. On the other hand, if too low a caustic concentration is employed, a sufficient purification or reaction with the impurities contained in the pulp, by the caustic soda solution, will not take place and the resulting product will not have undergone a sufficient purification and increase in tear test.

In other words, the concentration of caustic soda employed in the alkaline treatment of the "4-4" pulp is preferably maintained between two limits, namely, between a maximum concentration at which mercerization takes place, and a minimum concentration at which a sufficient increase in tear test of the pulp is not effected. These limits will vary somewhat, depending upon the exact 25 temperature or treatment employed and the different characteristics of the raw "4-4" stock undergoing the treatment.

After the purification treatment, the pulp is washed free from the alkaline treating agent and may then be bleached to a high degree of whiteness with the usual amount of hypochlorite bleach, without material injury to its strength or decrease in cellulose content. If a pulp of maximum whiteness is desired, the bleached pulp may finally be superbleached in a chlorine solution.

While I have indicated that the purification or refining treatment is ordinarily carried out at room temperature, I desire to have it clearly understood that lower than room temperature (say, 0° C. to 25° C.) may be employed in the treatment of the "4-4" pulp. Likewise, higher temperature (for example, 30° C. to 50° C.) and a correspondingly suitable concentration of caustic soda, may be employed in the treatment. Moreover, an alkaline liquor containing any other suitable alkaline compound or compounds, such as caustic potash and sodium sulphide, may be employed in the purifying treatment, if desired, one or more of these compounds being used to replace a portion or all of the caustic soda. For instance, substantially equivalent results to those previously outlined may be obtained by treating a "4-4" stock with a solution of sodium sulphide of somewhat higher concentration than a solution of caustic soda necessary for effecting the same results. Or white liquor such as utilized in a kraft mill for the production of kraft pulp, and containing sodium sulphide, sodium hydroxide, and a slight amount of sodium sulphate and sodium carbonate, may be frequently used with certain advantages. Where the caustic soda is replaced by a substantial proportion of

sodium sulphide, or in entirety thereby, mercerization of the alpha cellulose content of the pulp undergoing treatment is precluded, since sodium sulphide does not cause a mercerization of cellulose fiber. In certain cases it may be advantageous to incorporate into the cooking liquor, sulphur as such, or in the form of reducing sulphur compounds, such as sodium sulphide or sodium thiosulphate, in order to maintain a reducing condition in the mass during the purifying treatment. Such a condition, it is believed, tends to improve the yield and the qualities desired in the final product.

At any temperature, however, where a solution of caustic soda is employed for the purifying treatment, the maximum concentration of caustic soda which is preferably employed is below that at which mercerization occurs, and the minimum above that at which a sufficient increase in tear test is not effected. For optimum results in respect to alpha cellulose content in the finished product and in the tear test of the product, at a treating temperature of about 30° C., the minimum and maximum concentrations in a stock suspension of about 5% to 6%, are, respectively, about 100% to 175% caustic soda based on the weight of dry fiber.

It may be advantageous to employ a relatively small proportion of oxidizing agent or bleach prior to or in the alkaline treatment or purification of the "4-4" pulp, especially where the product is to be subsequently bleached. Such treatment renders the pulp more easily bleachable in the subsequent bleaching operation, and is especially desirable when the "4-4" pulp is especially high in ligneous and other coloring substance. Ordinarily, about 2% to 5% of 35% lime bleach ( $CaOCl_2$ ) based on the dry weight of pulp when used in the alkaline liquor is sufficient to render the pulp easily bleachable in subsequent operation. If desired, however, chlorine may be introduced into the alkaline treating solution to form the desired amount of sodium bleach in solution. Or the pulp may be treated for a relatively short period of time prior to the alkaline treatment, with an oxidizing agent, preferably in the form of a bleach or chlorine solution, depending upon plant expediency, about 2% to 4% of lime bleach, or 1% to 3% chlorine, being sufficient to render the difficulty removable non-alpha cellulose constituents contained in the pulp susceptible to removal in the subsequent treatment with the alkaline liquor. Or the pulp may be pretreated, after which it is preferably washed, and then treated with an alkaline liquor, as previously described. Of course, where an alkaline liquor containing a reducing agent such as sodium sulphide is employed, bleach or other oxidizing agent may not be added thereto.

In carrying out the treatment in accord-

ance with this invention, a "4-4" pulp produced by digestion in an acid sulphite liquor under the conditions hereinbefore described is washed substantially free of its digesting liquor and spent products of digestion and is preferably then screened prior to the alkaline treatment. It is then thickened and intimately admixed with an alkaline solution of caustic soda to a consistency of about 5% to 6%, the stock suspension containing about 100% to 175% of caustic soda, based on the weight of dry fiber. While a lower percentage of caustic soda may be employed in cases where the resulting pulp need not be of optimum tear test and of high alpha cellulosic content, in the practice of the present invention it is preferable to employ a caustic soda concentration between the limits indicated, so that a sufficient increase in tear test and purification of the fiber may be obtained without impairing or injuring its paper-making characteristics to any material extent, or in other words, without causing a substantial mercerization of the fiber. The alkaline treatment is carried out preferably while stirring or agitating the pulp so as to promote a uniform reaction, say, at room temperature (30° C.), and the purification may require thirty minutes to two hours, depending upon the characteristics of the particular stock undergoing treatment. The spent liquor contains not only a very high percentage of residual unconsumed caustic soda, but various organic substances removed from the sulphite pulp, as indicated. The large portion of spent liquor is reemployed in subsequent treatment of other pulp, and the chemicals in the remaining portion of such spent liquor may be recovered.

40 The washed pulp is of light color, not much different in appearance from the color of ordinary unbleached sulphite pulp. I present herewith a table indicating certain characteristics of a pulp which has been treated as hereinbefore described:

|                   |             |
|-------------------|-------------|
| Time of beating   | 100 minutes |
| Strength (Mullen) | 100-140     |
| Tear              | 240-270     |
| Pentosan          | 1.8-3%      |
| Alpha cellulose   | 90-94%      |

55 From the foregoing table, which represents the average of a number of tests on samples obtained from different batches of pulp treated with liquors of different concentrations of caustic soda, it will be seen that the Mullen strength of the pulp has undergone some reduction, but that the tear test has increased considerably. The treated fiber is no longer harsh and ratty; it resembles the feel of a strong rag sheet.

60 The purified fiber may now be bleached to a high whiteness without materially affecting its strength or tear, by treating it at a consistency of about 10% to 16% with about

5% to 10% of 35% lime bleach (CaOCl<sub>2</sub>), based on the dry weight of pulp. Precaution is taken to maintain a temperature not exceeding 90° F. in the bleaching operation, so as to preserve the maximum strength of fiber. If desired, a certain small proportion of caustic soda liquor may be added to the bleach liquor and pulp in the bleaching operation, to retard the bleaching reaction and thereby eliminate the possibility of lowering the alpha cellulose content or injuring the fiber strength of the stock, due to too violent bleaching. The bleaching period ranges from eight to twenty hours, depending upon the characteristics of the fiber undergoing treatment, and producing stock having a color of 95 to 100.

65 The stock thus bleached may be improved by a superbleaching operation. In superbleaching, the preferably washed and bleached high alpha cellulose stock is treated at a consistency of from 4% to 6% with about 0.2% to 0.5% chlorine, based on the weight of dry fiber. No effort need be made to control the temperature in superbleaching, which may approximate the temperature of the water available at the time. If it is desired to increase the rate of superbleaching, the temperature may be increased to a point not higher than 90° F. After superbleaching, the stock is treated with an anti-chlor, as, for example, a bisulphite solution, which serves to react with and to neutralize any residual traces of chlorine or hydrochloric acid present in the stock. The pulp is then washed free from reaction products, and may then be sent to a wet machine, from which it is taken off in sheet form, ready for shipment.

70 Due to its properties and the purifying treatment which it has received, the high alpha cellulose may be employed instead of rag fiber in the manufacture of high grade bond and ledger papers, or in the manufacture of the cellulose esters and the cellulose ethers, and for any other purpose where a substantially pure cellulose fiber is required.

75 Thus, by the practice of this invention, I am enabled to increase the tear test of the original sulphite fiber, at the expense of its strength, and in so doing to purify it and produce a product which is especially high in alpha cellulose. This is a very desirable occurrence, since the tear test and its accompanying quality of folding endurance is of extreme importance in high grade papers, whereas the Mullen or strength test is usually of secondary importance. This feature may be better understood from the fact that it is relatively easy to increase the Mullen or strength test of a paper sheet by suitable sizing. The sizing operation, however, does not affect the tear test so appreciably, so that it is a distinct advantage to increase the tear test at the expense of the strength of the pulp,

inasmuch as it is possible to increase the strength in subsequent treatment.

Moreover, paper made from the unbleached purified pulp as herein produced, because of its softness of sheet, is admirably adapted for many uses to which a harsh or ratty paper could not be put. For example, such paper may be employed for the production of artificial reed fiber such as employed in the manufacture of baby carriages, furniture, etc. Such a paper should have a high tear test, should be soft and yet firm, and should have sufficient porosity to permit its ready impregnation with glue or other chemical reagents.

Before concluding, it may be stated that, while I have specified certain concentrations of stock and treating compounds in order to more fully and adequately describe my invention, these concentrations may vary, depending upon plant equipment and conditions. That is to say, the plant equipment with which the practice of the present invention was carried out, permitted the treatment of "4-4" stock at a concentration of about 5% to 6%, most efficiently and successfully. On the other hand, a stock concentration of 10% or greater may be treated under other plant conditions. In such cases, the percentage of caustic soda or other alkaline compounds utilized in the purification may be correspondingly decreased. In other words, the determining factor in carrying out the treatment or purifying reaction resides in the concentration of the alkaline compounds in the liquor, even though for convenience these compounds may frequently be expressed in terms of dry fiber weight. Thus, a 5% stock suspension treated with 100% caustic soda based on dry fiber, represents a 5% caustic soda solution. Of course, if sodium sulphide or some other reagent which is less drastic or effective in its reaction than caustic soda is used, the percentage of such alkaline reagent must be increased, in order to produce a product substantially equivalent to that obtained by the use of caustic soda.

I do not herein claim the subject matter claimed in my Patent No. 1,635,637, issued July 12, 1927, which discloses the treatment of a sulphite pulp, such as herein described, with dilute alkaline liquors at elevated temperatures.

What I claim is:

1. A process which comprises digesting wood chips in an acid sulphite cooking liquor in which the free  $\text{SO}_2$  and combined  $\text{SO}_2$  are in approximately equal proportions of 3% to 4% each, under conditions of high temperature and pressure; separating the resulting pulp from the spent liquor of digestion; and treating such pulp, admixed with a solution of caustic soda to a stock consistency of about 5% to 6%, at about room temperature, for about thirty minutes to two hours, said

solution containing 100% to 175% caustic soda based on the weight of dry fiber.

2. A process which comprises digesting wood chips in an acid sulphite liquor having a combined  $\text{SO}_2$  content appreciably above that of a saturated solution of calcium bisulphite, and treating the resulting pulp at about room temperature with an alkaline solution containing sufficient alkali to react with and dissolve from such pulp a substantial proportion of its non-alpha cellulose constituent. 75

3. A process which comprises digesting wood chips in an acid sulphite liquor having a combined  $\text{SO}_2$  content appreciably above that of a saturated solution of calcium bisulphite and a free  $\text{SO}_2$  content approximately equal to its combined  $\text{SO}_2$  content, treating the resulting pulp with an oxidant, redigesting the oxidant-treated pulp at about room temperature with an alkaline solution containing sufficient alkali to react with and dissolve from such pulp a substantial proportion of its non-alpha cellulose content, and bleaching the alkaline-digested pulp. 80

4. A process which comprises pulping wood chips in an acid sulphite cooking liquor in which free  $\text{SO}_2$  and combined  $\text{SO}_2$  are present in approximately equal proportions of 3% and 4%, and treating the resulting pulp at about room temperature with an alkaline liquor containing sufficient alkali to react with and dissolve from such pulp a substantial proportion of its non-alpha cellulose content. 95

In testimony whereof I have affixed my signature.

GEORGE A. RICHTER.

105

110

115

120

125

130